# EUROPEAN PATENT SPECIFICATION

(11) **EP 1 806 392 B1**
(45) Date of publication and mention of the grant of the patent: **24.12.2008**
(21) Application number: 06013688.4
(22) Date of filing: 01.07.2006
(51) Int. Cl.: C11D 1/62, C11D 3/02, C11D 3/00

(54) **Stable aqueous esterquat compositions**
Stabile wässrige Esterquat-Zusammensetztungen
Composés quaternaires d'esters aqueuses stables

(30) Priority: 06.09.2005 EP 05019277
(43) Date of publication of application: 11.07.2007
(73) Proprietor: Clariant (Brazil) S.A., 04795-900 Sao Paulo SP (BR)
(72) Inventor: Lerch, Alexander Dr., 63571 Gelnhausen (DE); Scholz, Hans Juergen Dr., 63755 Alzenau (DE); Gallotti, Manlio, Sao-Paulo-SP CEP 01421-001 (BR); Nunes, George Italo Pitombeira, Sao-Paulo-SP CEP 04304-011 (BR); Kume, Gustavo, Sao-Paulo-SP CEP 05586-000 (BR); Barge, Claudia, Sao-Paulo-SP CEP 04022-002 (BR)
(74) Representative: Otto, Adalbert

(56) References cited:
- EP-A- 0 924 333
- EP-A2- 0 899 325
- DE-A1- 19 904 513

## Description

Quaternized fatty acid triethanolamine (TEA) esters and quaternized fatty acid methyldiethanolamine (MDEA) esters, which are commonly called "esterquats", are widely known in detergent industry. They provide a softening effect to textile materials, especially for cotton. These compounds are made by esterification of triethanolamine (TEA) or methyldiethanolamine (MDEA) with a fatty acid and subsequent quaternisation by reacting with a short chain alkyl sulfate or alkyl chloride. In the step of esterification of TEA esterquats, one, two or three hydroxyl groups may react with the fatty acid and accordingly commercially available esterquat compositions contain quaternized mono-, di- and tri-esterquats. For the case of MDEA esterquats, only mono and di-esterquats are present.

A problem of aqueous compositions containing these Esterquats is that the Esterquats are not stable over prolonged storage since they undergo hydrolysis. In order to prevent hydrolysis it is known to add alkali metal salts (JP 10-251 972).

It has now been found that also other metal salts are capable of preventing hydrolysis of esterquats.

The invention accordingly provides aqueous compositions consisting of an esterquat or mixtures thereof of the formula I wherein R is C₁-C₄-alkyl, preferably methyl, X has the same meaning as R or X is a group of the formula -C₂H₄OR², R¹ and R² are independently hydrogen or a group -COR³, R³ is C₇-C₂₁-alkyl or C₇-C₂₁-alkenyl and A is an anion, preferably chloride or methosulfate, and a metal salt, and optionally one or more auxiliary as defined in claim 1, which composition is free of alkali or alkaline earth metal salt, phthalocyanine metal complexes or phthalocyanine metal salts.

Since X in the formula (I) may be either an alkyl group R or a further hydroxyethyl group which may be esterified the claimed compositions contain either TEA esterquats or MDEA esterquats of the following formulas II and III:

The group -COR³ is preferably derived from natural occurring fatty acids such as capronic acid, caprylic acid, caprinic acid, lauric acid, myristiric acid, palmic acid, isostearic acid, stearic, oleic acid, eluidinic acid, arachinic acid, behenic acid and eruca acid. Preferred acids containing the group -COR³ are C₁₂/C₁₈ coco fatty acids, tallow fatty acid, fully or partially hydrogenated tallow fatty acid, palm fatty acid, partially or fully hydrogenated palm fatty acid or stearic acid.

As mentioned above the ester quats of formula II are present in the form of mixtures of the mono-, di- or triester of triethanolamine. Preferred mixtures are those which have 10 to 38 % by weight of the monoester (R¹ and R² being hydrogen), 46 to 63 % by weight of the diester (R¹ being hydrogen and R² -COR³) and 7 to 25 % by weight of the triester (R¹ and R² being -COR³). Especially preferred are also the following mixtures (all percentages are by weight):
Monoester: 18 - 22 %; diester 58 - 62 %; triester 18 - 22 %.
Monoester: 20 - 27 %; diester 53 - 60 %; triester 16 - 23 %.
Monoester: 29 - 37 %; diester 46 - 57; triester 7 - 14 %.

In the same way, the esterquats of formula III are present in the form of mixtures of mono and di-ester of methyldiethanolamine. Preferred mixtures are those which have from 1 to 70% by weight of monoester (R¹ being hydrogen), and from 30 to 99% by weight of the diester (R¹ being -COR³). Especially preferred are also the following mixtures (all percentages by weight): Monoester 2-60%; diester 35-98%, Monoester 2-40%; diester 60-98%.

The ester quat compositions accordingly to the present invention contain in general 0.5 to 30, preferable 2 to 24 and especially 4 to 22 % by weight of the ester quats of the formula II. In order to enhance the stability of these aqueous compositions a salt is added which is not an alkali or alkaline earth metal salt. The claimed compositions are free of such salts. Preferred salts are transition metal salts, more preferably are zinc and aluminium salts such as ZnSO₄, ZnCl₂ AlCl₃ or Al₂(SO₄)₃. These salts are present in an amount preferably from 0.002 to 10.0, preferably 0.03 to 5.0, and preferably 0.04 to 3.0 % by weight.

In a preferred aspect the compositions according to the invention are also free of rare earth metal salts, metal salts of fatty acids or chelating agents.

The compositions according to the present invention can be made by mixing the aqueous solution of the ester quats of formulas II and III final softener formulations with the salt. The salt can be added at any moment during the softeners process preparation and either in solid form or an aqueous solution. Heating and stirring is recommended for making the claimed compositions.
In order to make easier the preparation of the disclosed invention, a concentrated pre-mix containing the same molar and/or mass ratio between the ester quats and the additives can be prepared in order to be diluted up to 45 times. Other ingredients such as solvent, water or any ingredient that could be part of the final formulation may be added.

Depending on the intended use, the compositions according to the invention comprise, in addition to the mentioned compounds additives and auxiliaries which are customary and specific in each case selected from electrolytes, perfumes, perfume carriers, colorants, hydrotropes, antifoaming agents, other thickening agents, opacifiers, preservatives, , anti corrosion agents, co-surfactants and solvents.

In a second aspect of the invention the composition may be composed only of water, one or more esterquat of formula (I) and a metal salt, which composition is free of an alkali or alkali earth metal salt or phthalocyanine metal salts. The metal salt preferably is ZnSO₄, ZnCl₂, AlCl₃ or Al₂(SO₄)₃.

The compositions according to the invention are notable for a good storage stability and can be used as such as fabric softener or can be further diluted with water either at around room temperature or under heating .

### Examples

All the following compositions based on formula (II) have been prepared in the following way:
- I: Water was heated to 85°C
- II: addition of a varying amount of a 50 % solution of the salt as indicated and stirring for approximately 5 minutes with approximately 150 rpm
- III: addition of the ester quat (5 % active content referred to the final composition)
- IV: cooling under stirring within 30 minutes.

The ester quat used in all examples was a mixture of the following compounds:
16 - 24 % of a compound of the formula
58 - 64 % of a compound of the formula
16- 24 % of a compound of the formula

### Examples

For compositions based on TEA esterquats (formula II):

| | ester quat | ZnCl₂ | crossing point (days) |
|---|---|---|---|
| 1 | 5 % active matter | - | 53 |
| 2 | 5 % active matter | 0.13 | 63 |
| 3 | 5% active matter | 0.61 | 79 |
| | ester quat | AlCl₃ | crossing point (days) |
| 4 | 5 % active matter | 0.08 | 65 |
| 5 | 5 % active matter | 0.40 | 69 |

For compositions based on MDEA esterquats (formula III):
- I.: Water was heated to 45°C
- II.: Addition of the esterquat at 50°C
- III.: Cooling under stirring with approximately 150 rpm for 20 minutes
- IV.: Fast cooling under stirring for 10 minutes
- V.: Addition of a varying amount of a 50 % solution of the salt as indicated and stirring for approximately 5 minutes with approximately 150 rpm

| | ester quat | ZnCl₂ | crossing point (days) |
|---|---|---|---|
| 1 | 2% active matter | - | 28 |
| 2 | 2% active matter | 0.32 | 38 |

The stability profile of the formulations was monitored through storage at 45°C. The hydrolysis stability profile was analysed according to the amount of mono, di and triester analysed time to time. In the case of MDEA esterquats, it was analysed only the amount of mono and diesterquats. As hydrolysis happens the amount of monoester increases while the amount of diester decreases for both, TEA and MDEA estequarts. However, for TEA esterquats there is also a decrease on the triester amount. After a certain time the amount of monoester is higher than the amount of diester for TEA and MDEA esterquats and for TEA esterquats the triester is presented in low levels. The crossing point of the di and monoester curves was defined as the reference for comparison between the formulations. The later the crossing point, the lower the hydrolysis rate and, consequently, the more stable the formulation.

The results given above show that the addition of ZnCl₂ or AlCl₃ shifts the crossing point further as compared with the same formulation containing no salt. This indicates the positive effect on hydrolysis stability of these salts.

## Claims

1. Aqueous compositions consisting of an esterquat or mixtures thereof of the formula 1 wherein R is C₁-C₄-alkyl, preferably methyl, X has the same meaning as R or X is a group of the formula -C₂H₄OR², R¹ and R² are independently hydrogen or a group -COR³, R³ is C₇-C₂₁-alkyl or C₇-C₂₁-alkenyl and A is an anion, preferably chloride or methosulfate, a metal salt, and optionally one or more auxiliary selected from the group consisting of electrolytes, perfumes, perfume carriers, colorants, hydrotropes, antifoaming agents, thickening agents, opacifiers, preservatives, anti corrosion agents, co-surfactants and solvents, which composition is free of alkali or alkaline earth metal salt, phthalocyanine metal complexes or phthalocyanine metal salts.

2. Aqueous compositions as claimed in claim 1 wherein the esterquat is of the formula wherein R, R¹, R², R³ and A are as defined in claim 1.

3. Aqueous compositions as claimed in claim 1 wherein the esterquat is of the formula wherein R, R¹, R³ and A are as defined in claim 1.

4. A composition as claimed in claim 2 wherein the ester quat is of the formula II and is composed of 10 - 38 % by weight of monoester, 46 - 63 % by weight of diester and 7 - 25 % by weight of triester.

5. A composition as claimed in claim 3 wherein the ester quat is of the formula III and is composed from 1-70% by weight of the monoester and from 30-99% by weight of diester.

6. A composition as claimed in claim 1 wherein the total amount of ester quat of the formula II or of the formula III is from 0.5 to 30 % by weight.

7. A composition as claimed in claim 1 containing ZnCl₂, AlCl₃, ZnSO₄ or Al₂(SO₄)₃ as metal salt.

8. A composition as claimed in claim 1 containing 0.002 to 10 % by weight of the metal salt.

9. A composition as claimed in claim 1 containing one or more additives or auxiliaries.

10. A composition consisting of water, one or more esterquat of the formula I as defined in claim 1 and a metal salt, which composition is free of alkali or alkali earth metal salt or phthalocyanine metal salts.

11. A composition as claimed in claim 1 which is a concentrated pre-mix of the esterquat and metal salt.

## Patentansprüche

1. Wäßrige Zusammensetzungen, die aus einem Esterquat oder Mischungen davon der Formel 1 worin R für C₁-C₄-Alkyl, vorzugsweise Methyl, steht, X die gleiche Bedeutung wie R hat oder für eine Gruppe der Formel -C₂H₄OR² steht, R¹ und R² unabhängig voneinander für Wasserstoff oder eine Gruppe -COR³ stehen, R³ für C₇-C₂₁-Alkyl oder C₇-C₂₁-Alkenyl steht und A für ein Anion, vorzugsweise Chlorid oder Methosulfat, steht, einem Metallsalz und gegebenenfalls einem oder mehreren Hilfsstoffen aus der Gruppe bestehend aus Elektrolyten, Parfümen, Parfümträgern, Farbmitteln, Hydrotropen, Antischaummitteln, Verdickungsmitteln, Trübungsmitteln, Konservierungsmitteln, Korrosionsschutzmitteln, Cotensiden und Lösungsmitteln bestehen und frei von Alkali- oder Erdalkalimetallsalzen, Phthalocyanin-Metallkomplexen oder Phthalocyanin-Metallsalzen sind.

2. Wäßrige Zusammensetzungen nach Anspruch 1, worin das Esterquat die Formel worin R, R¹, R², R³ und A die in Anspruch 1 angegebenen Bedeutungen besitzen, aufweist.

3. Wäßrige Zusammensetzungen nach Anspruch 1, worin das Esterquat die Formel worin R, R¹, R³ und A die in Anspruch 1 angegebenen Bedeutungen besitzen, aufweist.

4. Zusammensetzung nach Anspruch 2, worin das Esterquat die Formel II aufweist und aus 10 - 38 Gew.-% Monoester, 46 - 63 Ges.-% Diester und 7 - 25 Gew.-% Triester besteht.

5. Zusammensetzung nach Anspruch 3, worin das Esterquat die Formel III aufweist und aus 1 - 70 Gew.-% Monoester und 30 - 99 Gew.-% Diester besteht.

6. Zusammensetzung nach Anspruch 1, worin die Gesamtmenge an Esterquat der Formel II oder der Formel III 0,5 bis 30 Gew.-% beträgt.

7. Zusammensetzung nach Anspruch 1, die als Metallsalz ZnCl₂, AlCl₃, ZnSO₄ oder Al₂(SO₄)₃ enthält.

8. Zusammensetzung nach Anspruch 1, die 0,002 bis 10 Gew.-% des Metallsalzes enthält.

9. Zusammensetzung nach Anspruch 1, die ein oder mehrere Additive oder Hilfsstoffe enthält.

10. Zusammensetzung, die aus Wasser, einem oder mehreren Esterquats der Formel I gemäß Anspruch 1 und einem Metallsalz besteht und frei von Alkali- oder Erdalkalimetallsalzen oder Phthalocyanin-Metallsalzen ist.

11. Zusammensetzung nach Anspruch 1, bei der es sich um eine konzentrierte Vormischung des Esterquats und des Metallsalzes handelt.

## Revendications

1. Compositions aqueuses constituées d'un composé quaternaire d'ester ou de mélanges de celui-ci de la formule 1 dans laquelle R représente un groupe alkyle en C₁ à C₄, de préférence un groupe méthyle, X a la même signification que R ou X représente un groupe de la formule -C₂H₄OR², R¹ et R² représentent indépendamment un atome d'hydrogène ou un groupe -COR³, R³ représente un groupe alkyle en C₇ à C₂₁ ou un groupe alcényle en C₇ à C₂₁ et A représente un anion, de préférence un chlorure ou un méthosulfate, d' un sel métallique, et éventuellement d' un ou plusieurs auxiliaires choisis parmi le groupe constitué d'électrolytes, de parfums, d'excipients pour parfum, de colorants, d'hydrotropes, d'agents antimousses, d'épaississants, d'opacifiants, d'agents de conservation, d'agents anticorrosion, d'agents cotensioactifs et de solvants, ladite composition étant exempte de sels de métaux alcalins ou alcalino-terreux, de complexes métalliques de phtalocyanine ou de sels métalliques de phtalocyanine.

2. Compositions aqueuses selon la revendication 1, dans laquelle le composé quaternaire d'ester est de la formule dans laquelle R, R¹, R², R³ et A sont tels que définis dans la revendication 1.

3. Compositions aqueuses selon la revendication 1, dans laquelle le composé quaternaire d'ester est de la formule dans laquelle R, R¹, R³ et A sont tels que définis dans la revendication 1.

4. Composition selon la revendication 2, dans laquelle le composé quaternaire d'ester est de la formule II et est constitué de 10 à 38 % en poids de monoester, de 46 à 63 % en poids de diester et de 7 à 25 % en poids de triester.

5. Composition selon la revendication 3, dans laquelle le composé quaternaire d'ester est de la formule III et est constitué de 1 à 70 % en poids de monoester et de 30 à 99 % en poids de diester.

6. Composition selon la revendication 1, dans laquelle la quantité totale du composé quaternaire d'ester de la formule II ou de la formule III varie de 0,5 à 30 % en poids.

7. Composition selon la revendication 1, qui contient du ZnCl₂, du AlCl₃, du ZnSO₄ ou du Al₂(SO₄)₃ comme sel métallique.

8. Composition selon la revendication 1, qui contient de 0,002 à 10 % en poids du sel métallique.

9. Composition selon la revendication 1, qui contient un ou plusieurs additifs ou auxiliaires.

10. Composition comprenant de l'eau, un ou plusieurs composés quaternaires d'ester de la formule I telle que définie dans la revendication 1 et un sel métallique, ladite composition étant exempte de sels de métaux alcalins ou alcalino-terreux ou de sels métalliques de phtalocyanine.

11. Composition selon la revendication 1, laquelle est un prémélange concentré du composé quaternaire d'ester et du sel métallique.
